

## UNITED STATES PATENT OFFICE.

DANIEL H. MELOCHE, OF DETROIT, MICHIGAN, ASSIGNOR TO EARL HOLLEY, OF DETROIT, MICHIGAN.

## MEANS FOR PROTECTING THE SURFACE OF CORES.

No Drawing.

Application filed March 31, 1922. Serial No. 548,475.

To all whom it may concern:

Be it known that I, DANIEL H. MELOCHE, a citizen of the United States, residing at 8450 Fourteenth St., Detroit, in the county of Wayne and State of Michigan, have invented certain new and useful Improvements in Means for Protecting the Surface of Cores, of which the following is a specification.

This invention relates to means for protecting the surface of dry sand cores, and relates specifically to the protection of dry sand cores from the erosive effect of molten cast iron, and is particularly adapted for use in conjunction with permanent iron molds in which iron castings are made.

The usual defect with such castings made in iron molds having sand cores is that the cored holes are rough, as particles of sand are carried by the flowing iron and the cast surface is thereby roughened. The object of this invention is therefore to produce a smooth surface in the cored hole.

I have discovered that an insulating coating of powdered magnesium oxide applied with a brush to an ordinary dry sand core, using gluten or any other satisfactory binder, is a satisfactory protection for the core. In addition, I may apply lamp black, carbon or other carbonaceous material superimposed above the coating of magnesium oxide.

The lamp black, carbon or other carbonaceous material doubtless acts to some extent as a lubricant, enabling the iron to flow easily

over the surface of the core. The magnesium oxide, on the other hand, being an insulator, prevents the molten iron from unduly raising the temperature on the surface of the sand core and thereby preventing the sand core adhering to the flowing metal.

What I claim is:

1. Means for protecting the surface of a dry sand core, consisting of the application of a substance, having the refractory qualities of magnesium oxide, mixed with a binder to the surface of the dry sand core.

2. Means for protecting the surface of a dry sand core from the action of molten cast iron, which consists in applying to the surface of the sand core a substance having substantially the refractory qualities of magnesium oxide.

3. Means for protecting the surface of a dry sand core from the action of molten cast iron, which consists in applying to the surface of the dry sand core magnesium oxide and superimposing a coating of a carbonaceous material.

4. Means for protecting a dry sand core from the action of molten iron, which consists in applying to the surface of the dry sand core first an insulating substance having substantially the refractory qualities of magnesium oxide and secondly a coating of a carbonaceous material.

In testimony whereof I affix my signature.

DANIEL H. MELOCHE.